

## UNITED STATES PATENT OFFICE.

WILLOUGHBY STATHAM SMITH, OF NEWTON POPPLEFORD, AND HENRY JOSEPH GARNETT, OF SEVENOAKS, ENGLAND.

## MAGNETIC ALLOY.

No Drawing.

Application filed January 10, 1924. Serial No. 685,432.

*To all whom it may concern:*

Be it known that we, WILLOUGHBY STATHAM SMITH, a subject of the King of Great Britain, residing at Benchams, Newton

5 Poppleford, Devonshire, England, and HENRY JOSEPH GARNETT, a subject of the King of Great Britain, residing at Lymne, Solefields, Sevenoaks, Kent, England, have invented a new and useful Improvement in

10 Magnetic Alloys, of which the following is a specification.

This invention relates to the production of alloys possessing a high magnetic permeability especially at low magnetizing

15 forces.

It is well known that it is desirable to add inductance to telegraphic and telephonic cables and this has before been done by wrapping around the core of the cable an iron

20 tape or wire.

Many research workers have been investigating the properties of various alloys, especially those of nickel and iron, with a view to discovering an alloy that should be

25 suitable for this purpose. In our researches we have found that an alloy may be made of nickel, copper and iron, which has a low hysteresis loss with a very high permeability at low magnetizing forces such as those

30 present in telegraphic and telephonic cables.

According to our invention we make an alloy of nickel, iron, copper and manganese, the nickel being at least 71%, the iron

35 about 20% and the copper about 5% with a small quantity of manganese to render the alloy more easy to forge.

In some cases, however, we may employ 15% to 25% copper with 49% to 71% nickel,

40 17% to 25% iron and manganese as before.

In order also to increase the electrical resistance of the alloy we preferably add to

45 it a fourth element which may be tungsten, chromium, silicon, vanadium, titanium, molybdenum or aluminium; the amount of this fourth element is small compared to the amount of copper and is preferably less than 1%, since the addition of more than 1% of this fourth element, though increasing the resistance, will impair the permeability of the alloy considerably.

We also preferably include a small amount of manganese to render the alloy more easy to forge.

The following are examples of alloys made in accordance with our invention:—

## No. 1.

An alloy consisting of:—

|           | Per cent. |
|-----------|-----------|
| Nickel    | 71.0      |
| Iron      | 18.5      |
| Copper    | 10.2      |
| Manganese | 0.3       |

has an initial magnetic permeability of 5500.

## No. 2.

An alloy consisting of:—

|           | Per cent. |
|-----------|-----------|
| Nickel    | 65.5      |
| Iron      | 17.0      |
| Copper    | 17.0      |
| Manganese | 0.5       |

has an initial magnetic permeability of 3200.

## No. 3.

An alloy consisting of:—

|           | Per cent. |
|-----------|-----------|
| Nickel    | 49.5      |
| Iron      | 25.0      |
| Copper    | 25.0      |
| Manganese | 0.5       |

has an initial magnetic permeability of 1700.

These alloys are sensitive to heat-treatment and should be annealed by heating to a considerable temperature and then cooled. This may conveniently be done by passing a wire or tape formed of the alloy through a tube heated electrically and allowing the wire or tape to cool rapidly as it issues from the tube.

If the correct temperature has not been used the magnetic properties will not be fully developed.

Example:—

Alloy No. 1, when heated to 890° C. and cooled in air has a permeability of 5300, but when heated to 730° C. only 3800.

Further, the annealing may be adjusted to give either:—

- (a) Maximum initial permeability, or
- (b) Maximum permeability at magnetic saturation, and
- (c) Low or high fields for magnetic saturation.

Moreover, when correctly annealed for high initial permeability, the alloys have

low hysteresis losses varying from 50 to 150 ergs per cubic centimetre with a maximum field of .25 C. G. S. units.

What we claim is:—

- 5 1. An alloy comprising nickel 49% to 71%, iron 17% to 25%, and copper 15% to 25%.
2. An alloy consisting of nickel 49.5%, iron 25%, copper 25% and manganese .5%.
- 10 3. An alloy consisting of nickel 65.5%, iron 17%, copper 17% and manganese .5%.
4. An alloy consisting of nickel 49% to 71%, iron 17% to 25%, copper 15% to 25% and a small quantity of manganese.
- 15 5. An alloy comprising nickel 49% to 71%, iron 17% to 25%, copper 15% to 25%, and a small quantity of manganese and tungsten.

6. An alloy comprising nickel 49% to 71%, iron 17% to 25%, copper 15% to 25% and tungsten. 20

7. An alloy comprising nickel 49% to 71%, iron 17% to 25%, copper 15% to 25% and a fourth element adapted to increase the electrical resistance of the alloy. 25

8. An alloy comprising nickel 49% to 71%, iron 17% to 25%, copper 15% to 25%, a small quantity of manganese and another element adapted to increase the electrical resistance of the alloy. 30

In testimony that we claim the foregoing as our invention we have signed our names this 14th day of December, 1923.

WILLOUGHBY STATHAM SMITH.  
HENRY JOSEPH GARNETT.